

# UNITED STATES PATENT OFFICE.

ZAKARIA N. BERGMAN, OF LOS ANGELES, CALIFORNIA, ASSIGNOR OF ONE-HALF TO  
HERMAN C. SCHMIDT, OF LOS ANGELES, CALIFORNIA.

## VARNISH AND PROCESS OF MAKING THE SAME.

1,307,805.

Specification of Letters Patent. Patented June 24, 1919.

No Drawing.

Application filed January 29, 1919. Serial No. 273,858.

To all whom it may concern:

Be it known that I, ZAKARIA N. BERGMAN, a citizen of the United States, residing at Los Angeles, in the county of Los Angeles and State of California, have invented new and useful Improvements in Varnish and Processes of Making the Same, of which the following is a specification.

My invention relates to a varnish, and it is the object of this invention to compound a varnish which is inexpensive, has excellent brushing qualities and leaves a durable, elastic layer of varnish on the goods to which it is applied.

My invention consists in the composition and in the steps of compounding the same hereinafter described and claimed.

In compounding my varnish, I use the following ingredients in the proportions stated:

$\frac{1}{2}$  gal. of boiled linseed oil.

1 quart of gloss oil which is a trade name applied to a varnish made of benzine and rosin or other inexpensive resin.

1 quart of benzine.

1 quart of coal oil.

1 pint of japan.

The above ingredients are thoroughly mixed together and a creamy paste prepared as follows is added thereto and thoroughly mixed.

$\frac{1}{6}$  of a pound of litharge (PbO).

A small quantity of water to make a paste with the litharge.

1 quarter of a pint of benzine.

The resulting varnish is thinner than the ordinary varnish and works freer under the brush, leaving no brush marks. The color is light straw, but when applied to the objects to be varnished it appears colorless.

35

Dyes or paint pigments may be added to this varnish as desired.

40

While I have described the preferred proportions of the ingredients to be used it will be understood by those skilled in the art 45 that the proportions may be varied without departing from the spirit of my invention as claimed.

I claim:

1. A varnish comprising boiled linseed oil, 50 rosin varnish, benzine, coal oil, japan, litharge and water.

2. A process of compounding a varnish comprising making a mixture of boiled linseed oil, rosin varnish, benzine, coal oil and 55 japan and adding thereto a mixture of litharge, water and benzine.

In testimony whereof I have signed my name to this specification.

ZAKARIA N. BERGMAN.

Copies of this patent may be obtained for five cents each, by addressing the "Commissioner of Patents, Washington, D. C."